

# UNITED STATES PATENT OFFICE.

PETER SCHMID, OF BASEL, SWITZERLAND.

## PROCESS OF PRODUCING FOAM OR FROTH BATHS FOR UNGUMMING SILK AND SILK-WASTES.

1,313,235.

Specification of Letters Patent. Patented Aug. 12, 1919.

No Drawing.

Application filed June 5, 1917. Serial No. 173,066.

*To all whom it may concern:*

Be it known that I, PETER SCHMID, a citizen of the Swiss Republic and resident of Basel, Switzerland, have invented a new 5 Process for Producing Foam or Froth Baths for Ungumming Silk and Silk-Wastes, of which the following is a full, clear, and exact specification.

It is known that the ungumming of silk 10 and silk wastes in all forms, as raw goods, spuns or tissues, was heretofore obtained by holding the goods for a certain time in boiling soap water or in lather bath produced by heating soap water or soap water containing 15 chrysalids.

I have now found an even cheaper process for producing a foam or froth bath for ungumming silk and silk wastes, which consists in heating, to the boiling point, a 20 weakly alkaline water bath containing only sericin as the foam producing substance.

Such an ungumming bath can, for instance, be prepared by adding a little alkali to the sericin water obtained by washing silk 25 previously treated with soap lather bath, so that an alkaline bath is obtained, containing

for instance for 100 kg. water, 25 gr. sodium carbonate and 200 gr. sericin. This bath constitutes, when transformed into froth or foam without addition of soap, a very effective and extraordinarily cheap ungumming bath wherein the sericin froth or foam carries the alkali.

What I claim is:

1. A process for producing a foam or froth 35 bath for ungumming silk and silk wastes, consisting in heating to ebullition a weakly alkaline water bath containing only sericin as a foam producing substance.

2. A process for producing a foam or froth 40 bath for ungumming silk and silk wastes, consisting in heating to ebullition a feeble watery solution of sodium carbonate containing only sericin as a foam producing substance.

In witness whereof I have hereunto signed my name this 12th day of May, 1917, in the presence of two subscribing witnesses.

PETER SCHMID.

Witnesses:

CARL O. SPAMER,  
OMAND RITTER.